

Nov. 19, 1929.

L. B. MILLER ET AL

1,736,615

METHOD OF BENEFICIATING MANGANESE ORES

Filed April 22, 1927

2 Sheets-Sheet 1



Fig. 1



Fig. 2

INVENTORS  
Leonard B. Miller and  
William G. Rinehart  
BY

Fay. Oberlin & Fay  
ATTORNEYS.

Nov. 19, 1929.

L. B. MILLER ET AL

**1,736,615**

## METHOD OF BENEFICIATING MANGANESE ORES

Filed April 22, 1927

2 Sheets-Sheet 2



Fig. 2.

### INVENTORS

Leonard B. Miller and  
BY William G. Rinehart

Fay Oberlin & Fay  
ATTORNEYS

## UNITED STATES PATENT OFFICE

LEONARD B. MILLER, OF CLEVELAND, OHIO, AND WILLIAM G. RINEHART, OF BATESVILLE, ARKANSAS, ASSIGNORS TO SAID MILLER

## METHOD OF BENEFICIATING MANGANESE ORES

Application filed April 22, 1927. Serial No. 185,779.

The present invention relates to a process for handling residual clays containing oxides of manganese and for processing such clays to recover the manganese oxides either in the 5 form generally known as manganese ores or in the form known as ferruginous manganese ores, the difference between the two types of ores being merely the proportions of manganese oxide to iron oxide in the finished or 10 processed product.

In clays of this nature containing oxide of manganese there is normally a small proportion of the oxides which are coarse and a major proportion of the oxides which are in 15 small particles and which are known as "fines". The coarse material or lumps, as it is called, occurs in these residual clays in such small percentages that only in rare cases can it be made available for use at commercially 20 economic cost and heretofore no way has been known to make commercially available the largely preponderating quantity of fines for the reason that no practical method for 25 their beneficiation and separation from the clays has been known.

The present process will beneficiate and make the oxides economically available for commercial and metallurgical use and this process broadly consists in taking the clays 30 and first passing them into a soaking pit and thereafter passing them through a log washer arranged in a particular fashion at the end of which part of the process the material is picked or separated and the lumps made immediately available. The remainder of the 35 material containing all of the fines is then passed through a series of washing and concentrating units and washed continuously with an excess of water at all stages until the impurities have been substantially eliminated and the available fines are then removed and preferably processed by means of heat so as to remove not only the free or 40 meteoric water, but also the water of crystallization, and thus the finished material is in the form of manganese ore or ferruginous manganese ore. To the accomplishment of the foregoing and related ends, said invention 45 then, consists of the means hereinafter fully

described and particularly pointed out in the claims.

The annexed drawings and the following description set forth in detail certain means and one mode of carrying out the invention; 55 such disclosed means and mode illustrating, however, but one of various ways in which the principle of the invention may be used.

In said annexed drawings:

Figs. 1 and 1A are diagrammatic elevation- 60 al views of apparatus for carrying out the present process; and Figs. 2 and 2A are dia- grammatic plan views of such apparatus.

In carrying out the present process of beneficiating manganese oxides, the oxide bearing 65 clay as it is mined is first transported to and dumped into a soaking or saturation tank or pit 1 to which water is continuously added, the water being sufficient in quantity to saturate and substantially emulsify the clay so far as 70 is practicable in this initial step and the oxide bearing clay is normally added to and removed from the pit as a continuous operation.

It is, of course, understood that this first 75 preliminary soaking step could be accomplished by any satisfactory mechanism such as a mixing device with agitating mechanism and if a device of this type is employed, the material would be treated either in batches or continuously.

From this soaking pit the partially saturated mineralized residual clay is removed 80 and passed into a log washing unit 2 in which it is further treated by adding continuously an excess of water from pipe 3 and 85 in this log washer the material is continuously stirred or agitated by the use of paddles. This agitation and disintegration of the material is aided by the introduction of pieces of rock or iron or steel balls of suitable size. 90 In adding water to the material in the log washer, the water should be sufficient in quantity to further liquefy the original muddy solution and accelerate the solution of the clay and its gradual separation from 95 the metallic oxides which are present. The log washer preferably used in the present process is built as shown with higher sides 3 at the low end 4 or end for the reception of the material than the height of the dis- 100

charge aperture 5 which is located at the high end and thus the ores are preserved instead of passing off with the excess water as would be the case in a standard form of log washer in which the discharge end is higher than the intake end. From the log washer 2 the material is discharged into a screening or sizing apparatus 6 preferably into the end of a revolving screen cylinder into which are introduced additional quantities of clear water from pipe 8 sufficient to wash the fine material off and separate it from the coarse material, the fines thus passing through the holes in the screen and being carried off by a flume or chute 9 to a settling tank 10 or like unit while the coarse materials pass out of the discharge end of the screen and are deposited on a picking belt or conveyor 11 where they are sorted. These coarse materials are comprised of lump ore, lump rock and undissolved ore bearing clay in a form which is usually termed "clay balls". The lump ore is hand picked and saved for either shipment direct, or for further processing in the nature of sintering. The clay balls are returned to the log washer preferably by conveyor belt 15 and the lump rock may also be returned in such quantities as may be found desirable to aid in the disintegration being carried on in the log washing unit. The returned clay balls are thus further agitated and broken up in the log washer and as finely broken up pass through the entire process in due course.

The further processing of the material deals only with the fines which pass directly into the settling chamber 10 from the sizing screen and this settling tank or chamber 10 is formed with a discharge chute 17 at one end. Water is continuously added to the chamber preferably near the bottom thereof through a pipe 18 so as to agitate and keep the material stirred up and partially in suspension and the water as it overflows carries with it mud and lighter materials to a mud pond or waste material pond through a chute 19 while the heavier materials which contain the fines of desirable ores settle to the bottom of the tank and are removed therefrom by a conveyor 20 which carries these materials to the rear end of the tank against the flow of water from pipe 18 as it is forced into the tank and through a chute or flume and into a second log washer 22 which is located below and beyond the settling tank as shown in the drawings. In this settling chamber, a great deal of impurities such as the lighter clays and soil is removed, and the ore and the metallic oxides which are passed into this log washer and are largely separated from the original mother clay but are still so contaminated or mixed with clay as to necessitate further processing.

In this second log washer 22, which is of conventional design, the fines with the impurities still present, are washed and agi-

tated and clear water is continuously added to this log washer to remove impurities. The overflow from this washer leads to another settling tank 25 where additional clear water is added and the clay bearing water is removed from the top of the tank through a chute 26 to the mud pond while the very fine oxides are removed by a conveyor 27 and transferred to the ore stream in the log washer and added to the oxides therein.

The ore stream from the washer passes out from the high end thereof through a chute 30 into a storage box or device 31 which has a discharge chute 32 connected to an elevating mechanism 33. The material then passes out through the elevator and into a screening device 34 and the fine part of the material passes out through the meshes of the screen and through a suitable chute 35 into a gang bin or settling tank 36 while the coarser particles of the material which are too large to pass through the meshes of the screen, pass out from the end of the screen cylinder into a hopper 50 which feeds them through a crusher 37. From the crushing rolls, the material passes back into the lower part of the elevator by means of a chute 51 so that the crushed material can thus pass up through and into the screening cylinder again until all of the material is brought to a uniform or satisfactory size. Water is added to the material in the screening cylinder from pipe 38 so as to aid in washing the fines through the cylinder and also to aid in dissolving or washing off such clays as may be present at this stage of the process. The material, while in the gang bin or settling chamber 36 is further treated by adding clear water at the bottom of the chamber through pipes 52 so as to agitate and keep the material moving, and the excess water from the gang bin flows off at the top of the bin through suitable chute 39 to the mud or waste pond.

The metallic oxides which are now practically free from clay are removed from the gang bin by a suitable conveyor 40 and are passed through a chute or delivery mechanism 41 to a series of concentrating tables 42 on which they are separated so far as practicable from particles of foreign material such as lime or silica which up to this stage of the process have not been separated from the metallic oxides. This table separation is aided by the use of additional clear water from pipes 43 as in every stage of the process. From the concentrating tables the substantially purified metallic oxides are passed into a storage bin 44 by means of a suitable sump 45 and pump 46, and from the storage bin the processed material which is now in the form of substantially pure oxides of manganese and iron is removed.

The further steps as shown by the apparatus disclosed are employed mostly for preparing the metallic oxides for shipment to

distant points. If the material could be used at some nearby place, the further processing might be of a different nature, but for distant shipments, the material from the last storage bin 44 is preferably passed through a drying and sintering cylinder 47 where both the free or meteoric water and the water of crystallization are substantially removed. The dried or burned material from the sintering cylinder is then passed into the final storage bin 48 from which it is shipped in the form of manganese or ferruginous manganese ores.

In carrying out the present process for the beneficiation of the raw material, the first real step in the process is to soak or saturate the material and then to agitate it or pass it through a log washer in the presence of an excess of clear running water until it is in condition to be sized and picked for the removal of the coarser lumps of ore which form a fairly definite percentage of the total oxides which may be removed.

The second general step in the process is then to beneficiate the fines until substantially all of the impurities are removed and this is accomplished by passing the fine material through a series of settling and washing chambers in each of which an excess of clear water is added so as to dissolve and wash off in each stage as much of the impurities as is possible.

It has been found practical to accomplish this result by first passing the fines into a settling chamber in which they are continuously washed and agitated and then into a second log washer with its settling tank and conveyor mechanism by which material is returned to the washer and then passing the material by means of the elevating mechanism through the sizing screen and into the gang bin and in this step the coarser parts of the material are crushed and returned to the screen so that the material as it reaches the gang bin is properly sized.

At this stage the material is reduced to substantially metallic ore together with such impurities that water will not remove such as lime, silica, etc., and the removal of this is accomplished in the next step by means of the concentrating tables and the material as passed into the storage bin from the concentrating tables is in the form of substantially pure metallic oxides, which, of course, are mixed with water and are thus in a liquid state and this liquid is preferably of a consistency such that it may be handled by a pump and thus moved up into a storage bin. The metallic oxides of this nature may be found to be either such as are known as manganese ores or they may be such as are known as ferruginous manganese ores and this will depend entirely upon the nature and proportion of the two types of the original clay which was mined.

To reduce the weight and make them available for shipment to steel furnaces and the like, where material of this type is used, the liquid material is passed through a drying or sintering cylinder so as to eliminate the water contained and it has been found advisable to use a type of plant which will not only dry out the free water, but will also eliminate or reduce the water of crystallization as far as possible.

The finished materials of either type are then passed into the final storage bin in a dry state from which shipments may be made. The lumps of manganese oxide which were removed at the picking belt are brought to the final storage bin or to a similar bin by separate mechanism and it has been found that the lump ores, as they are known, are normally higher in the manganese contained as compared to the iron contained than are the fines and the lump ore is thus ordinarily found to be of a character such that it is properly sold as manganese ore while in most instances the fines are of the character which is commonly known as ferruginous manganese ore.

It is necessary through the entire process to use an excess of clear water in every step and without continuous addition of excess quantities of clear water it has been found practically impossible to concentrate the desirable oxides out of the original clay.

In residual clays of the nature used in the present process such as are found in quantities in Arkansas, the percentage of manganese ores present in the clay varies from ten to twenty per cent of the original mined product and in the ore content from the original clay, the lump ore is usually not over from 2 to 4 per cent of the total ore to be recovered, while the fines run from 96 to 98 per cent of the total amount of ore in the clay. The present process and the apparatus for carrying out such process as shown in the drawings, are relatively simple inasmuch as the material passes largely by gravity from the original soaking pit to the second settling tank and after one elevator mechanism passes again through the concentrating tables to the second elevating mechanism in the form of a pump. The fresh water is added in each of the washing and settling stages, and ordinarily is added always at the bottom of the chamber so as to have an agitating and rolling effect upon the material being treated.

Other modes of applying the principle of our invention may be employed instead of the one explained, change being made as regards the means and the steps herein disclosed, provided those stated by any of the following claims or their equivalent be employed.

We therefore particularly point out and distinctly claim as our invention:

1. The method of beneficiation of manga-

130

nese oxide ores consisting of first soaking and washing the ore and sorting the lump from the fines, then removing the clay and dirt by washing and agitating the fines through a series of steps all in the presence of an excess of clear water, crushing the obtained ore to a uniform maximum size, and mechanically freeing the ore from foreign materials.

2. The method of beneficiation of manganese oxide ores consisting of first soaking and washing the ore and sorting the lump from the fines, then removing the clay and dirt from the fines, by repeated agitation, and soaking and washing in the presence of an excess of clear water, reducing the ore to a uniform maximum size and washing the ore as it is being sized, mechanically concentrating and freeing the obtained ore from other impurities.

3. The method of beneficiation of manganese oxide ores consisting of first soaking and washing the ore and sorting the lump from the fines, passing the fines into a settling chamber and washing them therein by adding an excess of clear water, further removing of impurities by washing the product in a log washer and simultaneously adding an excess of clear water, again passing the material into a settling chamber and agitating with an excess of clear water to remove the remainder of the clay and dirt, sizing the material in the presence of clear running water, again settling and cleansing the sized material in a tank to which an excess of clear water is added, and passing the cleaned materials to concentrating tables for the removal of other materials.

Signed by us this 7th day of April, 1927.

LEONARD B. MILLER.

WILLIAM G. RINEHART.

40

45

50

55

60

65